

# United States Patent Office

3,198,660

Patented Aug. 3, 1965

1

3,198,660

## TREATMENT OF CELLULOSIC TEXTILE FABRICS WITH BISFORMAMIDE-FORMALDEHYDE AD- DUCTS

Sidney L. Vail and John G. Frick, Jr., New Orleans, and  
Wilson A. Reeves, Metairie, La., assignors to the United  
States of America as represented by the Secretary of  
Agriculture

No Drawing. Filed June 20, 1962, Ser. No. 204,013

6 Claims. (Cl. 117—139.4)

(Granted under Title 35, U.S. Code (1952), sec. 266)

A non-exclusive, irrevocable, royalty-free license in the  
invention herein described, throughout the world for all  
purposes of the United States Government, with the  
power to grant sublicenses for such purposes, is hereby  
granted to the Government of the United States of  
America.

This invention relates to the treatment of cellulosic textile  
materials to produce textiles having improved properties.  
More specifically, the present invention relates to  
new textile treating agents and a method of treating cellulosic  
textile fabrics with these agents whereby the fabrics  
are rendered resistant to wrinkling, have improved resiliency,  
and possess wash-and-wear properties. Moreover,  
the finishes produced from the new textile treating agents  
of this invention were found to be extremely durable.  
These finishes were found to effectively resist hydrolytic  
removal under conditions that remove the finishes based  
on the commonly used N-methylol treating agents.

In general, the production of wrinkle resistant and  
wash-and-wear fabrics has been accomplished by the use  
of di- and polyfunctional N-methylol finishing agents.  
These agents are generally formed by the addition of  
formaldehyde to ureas (cyclic or straight chain), melamine,  
and other similar type compounds. However, it is  
well known that finishes produced from these agents  
are fairly easily removed by repeated washing procedures  
which employ moderately strong acidic solutions, that is,  
the "souring" step used in most commercial launderings.  
After such treatments, it is often found that the treated  
fabric has lost the finish and the desired wrinkle resistance  
and wash-and-wear properties. Consequently, these  
treating agents cannot be used to produce acceptable  
wash-and-wear cellulosic fabrics which are to be subjected  
to these, or similar, hydrolytic conditions.

In the recent work [American Dyestuff Reporter, 50,  
No. 12, 29 (1961)] it was shown that N-methylolamides  
formed from acetamide and formamide produced finishes  
which were much more resistant to acidic hydrolysis than  
the finish derived from the N-methylol derivatives of  
ureas. More recently it was found that N-methylol derivatives  
of bisamides would form finishes on cellulosic  
fabrics which would prove to be highly resistant to acidic  
hydrolysis.

In general, alkaline hydrolysis is somewhat less detrimental  
than acidic hydrolysis under the normal conditions  
encountered in use.

A primary object of the present invention is to provide  
methylol derivatives of bisamides which have outstanding  
characteristics as treating agents for cellulosic textiles.

Another object of the invention is to provide a process  
for the treatment of textile fabrics, composed mainly of  
cellulose, with a new type of methylolamide treating  
agent, whereby the finished fabric acquires the properties  
of increased resiliency and wrinkle resistance. It is  
furthermore an object of this invention to provide such a  
treatment whereby the finish produced is resistant to  
harsh conditions of acidic hydrolysis and is not susceptible  
to alkaline hydrolysis. A further object of the present  
invention is to provide a finished fabric of the above

2

desirable properties without suffering excessive fabric  
damage.

In general, these and other objects of the invention are  
accomplished by treating the cellulosic textile with an  
aqueous solution containing the methylol derivatives of  
bisamides having the following structure:



wherein  $n$  is an integer of one to four. As is evident  
from the above structural formula the bisamides suitable  
for use in the present invention must be bisformamides  
having two amido hydrogens available for addition  
of formaldehyde. These bisformamides can be obtained  
economically by procedures well known to those  
skilled in the art. For example, methylenebisformamide  
can be prepared conveniently by heating formaldehyde  
and formamide. The other bisformamides can be prepared  
by diformylation of the particular diamine with  
formamide, alkyl formates, or other similar formylating  
agents. It is believed that the bisformamides are capable  
of the addition of two molar equivalents of formaldehyde  
to form a difunctional, or N,N'-dimethylol, derivative.

The N-methylol derivatives of the bisformamides used  
for the treatment of the cellulosic textile in the process  
of this invention can be conveniently obtained by the  
reaction of formaldehyde with the bisformamide of the  
above-described structure in aqueous media under slightly  
alkaline conditions. It is preferred to employ about three  
molar equivalents of formaldehyde to one of the bisformamide.  
A smaller quantity of formaldehyde can be used, but it has been found that the smaller quantity  
(two molar equivalents of the stoichiometric quantity of  
formaldehyde to produce complete methylation based  
upon the number of reactive hydrogens available in the  
particular bisformamide) does not produce a treated  
fabric with the highest wrinkle recovery angle. An  
amount of formaldehyde significantly in excess of the  
three to one ratio can also be employed, but it is inefficient  
and uneconomical to use such a large excess. The  
other conditions of this reaction are well known in the  
trade. Generally, heating the aqueous solution of the  
bisformamide and formaldehyde at 60° C. for 30 minutes  
is sufficient to achieve formation of the methylol derivatives.  
The reaction products thus produced are water  
soluble. The solution can be used as is or can be diluted  
with water for treatment of the cellulosic material.

Prior to application of the agent to fabric, an acidic  
substance or a substance producing acidity at elevated  
temperatures is added to the diluted solution to serve  
as a catalyst. The concentration of the reactants, i.e.,  
the bisformamide-formaldehyde adduct plus the excess  
or unreacted formaldehyde, can be varied depending on  
the particular textile processing conditions used, the type  
of textile being treated, and the properties desired in the  
finished textile. Generally, it is preferred to use from  
about 5% to 20% by weight of the reactants in the  
diluted treating solution. The catalysts which may be used  
are well known in the trade. Magnesium chloride, zinc  
fluoborate, and zinc nitrate are examples of particularly  
suitable catalysts. From about 0.5% to about 5% by  
weight of the acidic catalyst is generally preferred.

Treatment of the cellulosic textile material is carried  
out by standard procedure. The textile is thoroughly  
wetted with the above-described treating solution; the  
excess liquid is mechanically removed, and the wetted  
textile is dried and cured. Following the curing operation  
it is preferable, but not absolutely necessary, to water-  
wash the treated textile in an alkaline solution to remove  
any unreacted materials.

The processes of this invention can be used to treat substantially any hydrophilic fibrous cellulosic material such as cotton, rayon, ramie, jute, and the like which can be impregnated with a liquid, dried, and cured.

The following examples are given by way of illustration and not by way of limitation of the invention. The detailed procedures given below in the examples are illustrative, and are not the only or specific conditions for the production of an acceptable finished textile. Many variations or additions within these procedures can be made, as will be readily apparent to those skilled in the art. In the examples, all parts and percentages are by weight unless noted otherwise. The fabrics were tested by the following methods: Wrinkle recovery angle, Monsanto method, American Society for Testing Materials (ASTM) test D1295-53T; tearing strength, Elmendorf method, ASTM test D1424-59.

### EXAMPLE 1

1,3-propanebisformamide was prepared by refluxing 74 grams of 1,3-propanediamine and 300 grams of methyl formate. The excess methyl formate and any low boiling products were removed by distillation. The resultant yellowish oil was further concentrated by a vacuum distillation at 5 mm. with a maximum pot temperature of 175° C. The 1,3-propanebisformamide contained 21.36% nitrogen and was found (by osmometer) to have a molecular weight of 130 (theory for  $C_5H_{10}N_2O_2$ : 21.53% nitrogen and 130 for the molecular weight).

### EXAMPLE 2

To five grams of the bisformamide was added a slightly alkaline, aqueous solution of formaldehyde such that the molar ratio of formaldehyde to the bisamide was 3:1. The solution was either kept at room temperature for 18-24 hours or heated to 50-60° C. for about two hours. Then, two grams of magnesium chloride hexahydrate was added (final concentration was 4%) and the weight of the solution adjusted to a total of 50 grams by the addition of water. A sample of 80 x 80 cotton print fabric was dipped in the treating solution and padded to give about 70-80% increase in weight of the fabric. The wet fabric was dried seven minutes at 60° C. and cured for three minutes at 160° C. This treatment was followed by a wash in warm alkaline water, with a non-ionic detergent added, and then tumble drying. Using this general procedure, with variations noted where appropriate, the following bisformamides were used to produce wrinkle resistant fabrics, the properties of which are shown in Table I:

Example 2A. Methylenebisformamide.

Example 2B. Ethylenebisformamide, with a 2:1 molar ratio of formaldehyde to the bisformamide.

Example 2C. Ethylenebisformamide.

Example 2D. Ethylenebisformamide, with a catalyst of 0.8%  $Zn(BF_4)_2$ .

Example 2E. 1,3-propanebisformamide (as prepared in Example 1).

Table I.—Warp properties of treated fabrics

| Example          | Wrinkle Recovery Angle, deg. | Tearing Strength, g. |
|------------------|------------------------------|----------------------|
| 2A               | 136                          | 560                  |
| 2B               | 115                          | 640                  |
| 2C               | 124                          | 587                  |
| 2D               | 121                          | 580                  |
| 2E               | 122                          | 827                  |
| Untreated Fabric | 75                           | 1,087                |

### EXAMPLE 3

The durability of the finishes to acidic hydrolysis was tested by heating the fabrics for thirty minutes at 80° C. in a solution containing 1.5% phosphoric acid and 5% urea. Also, a fabric prepared in the usual manner from a dimethylolurea solution was hydrolyzed for comparison purposes. The results of the hydrolysis test are given in Table II.

Table II.—Acid hydrolysis of amide finishes

| Agent type       | Percent of original nitrogen retained after hydrolysis |
|------------------|--------------------------------------------------------|
| As in Example 2A | 89                                                     |
| As in Example 2C | 100                                                    |
| As in Example 2E | 90                                                     |
| Dimethylolurea   | 5                                                      |

### EXAMPLE 4

The durability of a representative finish, prepared from a methylenebisformamide, to basic hydrolysis was tested by heating the fabric for thirty minutes at 80° C. in a solution containing 1% sodium carbonate. The fabric (as in Example 2A) retained 98% of the original nitrogen after hydrolysis under these conditions.

We claim:

1. A process for producing a wrinkle resistant cellulosic textile material that is resistant to acidic and to basic hydrolysis comprising impregnating a cellulosic textile material with an aqueous material containing from 5 to 20% by weight of the reaction product of at least 2 moles of formaldehyde and 1 mole of a bisformamide represented by the formula:



wherein  $n$  is an integer of from 1 to 4, and from 0.5% to 5% by weight of an acidic catalyst and heating the thus impregnated cellulosic textile material to dry and cure it.

2. The process of claim 1 wherein the bisformamide is methylenebisformamide.
3. The process of claim 1 wherein the bisformamide is ethylenebisformamide.
4. The process of claim 1 wherein the bisformamide is 1,3-propanebisformamide.
5. The process of claim 1 wherein the acidic catalyst is magnesium chloride.
6. The process of claim 1 wherein the acidic catalyst is zinc fluoborate.

### References Cited by the Examiner

#### UNITED STATES PATENTS

|           |       |                            |
|-----------|-------|----------------------------|
| 2,562,161 | 7/51  | Epelberg et al.            |
| 2,765,336 | 10/56 | Hurwitz et al. 260-561     |
| 2,819,307 | 1/58  | Albert 260-561             |
| 2,985,544 | 5/61  | De Monterey et al. 117-143 |
| 2,985,546 | 5/61  | Leavitt 117-143            |
| 3,024,135 | 3/62  | Sookne et al. 117-139.4    |

### OTHER REFERENCES

- 65 J. Org. Chem., vol. 27 (1962), 260-561 (pp. 1062-70 pertinent).

WILLIAM D. MARTIN, Primary Examiner.

IRVING MARCUS, Examiner.